

March 2, 1954

R. F. HAUSER

2,671,039

MAGNESIUM DIE CASTING ALLOY AND PROCESS

Filed May 2, 1946

*Fig. 1*



*Fig. 2*



INVENTOR

RICHARD F. HAUSER

BY *Herbert L. Daigle*  
ATTORNEY

## UNITED STATES PATENT OFFICE

2,671,039

MAGNESIUM DIE CASTING ALLOY AND  
PROCESS

Richard F. Hauser, Bergenfield, N. J., assignor to  
Bendix Aviation Corporation, Teterboro, N. J.,  
a corporation of Delaware

Application May 2, 1946, Serial No. 666,759

4 Claims. (Cl. 148—21.90)

1

The present invention relates to a novel magnesium die casting alloy and process for producing such an alloy, and is a continuation in part as to all common subject matter of my copending application Serial No. 575,568 filed January 31, 1945, for Magnesium Die Casting Alloy and Process, now abandoned.

An object of the invention is to provide a magnesium alloy having excellent die casting characteristics, whereby both light and heavy sections may be die cast with slight tendency towards hot cracking during the die casting process and only moderate tendency towards internal porosity in the heavy sections.

Another object of the invention is to provide a magnesium alloy having superior corrosion resistance due in part to its manganese content and also to its low impurity content caused by the settling out in large part of such impurities through the novel method employed in preparing the alloy.

Another object of the invention is to provide a novel process for preparing a magnesium alloy for use in die casting.

Another object of the invention is to provide a novel method of preparing a magnesium alloy in which there is added to a magnesium-manganese alloy an amount of aluminum to decrease the solubility of the manganese in the alloy so as to precipitate a portion of the manganese out of solution tending to cleanse the melt of suspended iron particles while the temperature of the melt is maintained sufficiently high so as to prevent reduction of the manganese below a predetermined desired value.

Another object of the invention is to provide a novel magnesium alloy having a substantially homogeneous equi-axed grain structure.

Another object of the invention is to provide a novel heat treatment or artificial aging process for increasing the yield strength and hardness of die castings of this alloy.

Another object of the invention is to provide a process for causing an equi-axed grain structure to occur with resultant improved ductility and stability to the material. By the term "equi-axed" is meant the approximate equal dimensions of the grain with relation to their own axes and in relation to each other.

Other objects and advantages of this invention are set forth in the following description and the novel features thereof are pointed out in the appended claims. The disclosure, however, is illustrative only and changes may be made therein within the principle of the invention to the full extent indicated by the broad and general meanings of the terms in which the appended claims are expressed.

In Figure 1, there is illustrated a photo-micrograph of a typical grain structure obtained in

2

this alloy in the as cast condition and before aging.

In Figure 2, there is illustrated a photo-micrograph of a typical grain structure obtained in this alloy after the heat treatment or artificial aging process explained hereinafter and forming the subject matter of the present application.

Specifically, as an example of my invention, 10 the alloy is prepared by melting a binary magnesium-manganese alloy containing approximately 1.5% manganese by weight, and to the molten metal adding 1.00% to 1.5% aluminum by weight at approximately 1250-1350 degrees

15 Fahrenheit.

The addition of this amount of aluminum will 20 decrease the solubility of the manganese in the magnesium to between .5% and 1.0% by weight. The melt is held at this temperature for an appreciable period depending upon size of melt, for example, a minimum of fifteen minutes for a thousand pound melt, so that the manganese which is precipitated out of solution tends to cleanse the melt of suspended iron and other particles by causing them to sink to the bottom of the melt due to agglomeration of these particles to the precipitated primary manganese.

This action is not to be confused with the heretofore known settling process in which the precipitation of manganese depends primarily upon 30 holding the melt for long periods of time at relatively low temperatures. In the instant process the temperature of the alloy should never be allowed to drop below 1250 degrees Fahrenheit before being cast or frozen, as such a decrease in temperature below 1250 degrees Fahrenheit during the settling process might cause an adverse reduction of the manganese below the specified desired minimum of .5%. It is important to retain at least this amount of manganese in order to still further increase the corrosion resistance of the alloy.

The magnesium alloy thus obtained will have 40 an aluminum content by weight of between 1.0% to 1.5%, a manganese content by weight of not less than a .5% minimum and impurities or other ingredients by weight not in excess of a .3% maximum.

Upon completion of the settling process, the 50 thus-cleansed magnesium-manganese-aluminum alloy is removed and may be directly die cast or may be cast into pigs for convenience in handling. In the latter event, the pigs, as desired, are reheated to a temperature of between 1250 degrees and 1350 degrees Fahrenheit for pouring 55 into a die casting mechanism of conventional type.

Due to the short time for diffusion during solidification, sufficient deviation from equilibrium conditions are attained to permit a small

amount of the hardening material or eutectic to be retained at the grain boundaries of the solidified metal. Precipitation of the eutectic, an aluminum-magnesium compound, is later accentuated by a novel artificial aging process explained hereinafter. However, the amount of this material in the grain boundaries is not sufficient to cause excessive hot shortness or embrittlement of the die castings at elevated temperatures, since the aluminum content is preferably maintained at a value not in excess of 1.5% by weight. It has been found that with an aluminum content in excess of 1.5%, hot-shortness or embrittlement at elevated temperatures becomes so pronounced that it would be very difficult to make certain die castings without hot-cracking occurring as the casting is ejected from the die.

It is important, however, that the aluminum content of the alloy be maintained at a minimum of 1.0% or good mechanical properties will not be obtained in the subsequent die castings after the heat treatment or aging process and internal porosity will be increased to such an extent as to cause the castings to be unsound.

This alloy has the following composition:

|                                          |             |
|------------------------------------------|-------------|
| Aluminum                                 | 1.0-1.5%    |
| Manganese                                | 0.5-1.0%    |
| Nickel                                   | 0.005% max. |
| Iron                                     | 0.005% max. |
| Copper                                   | 0.05% max.  |
| Silicon                                  | 0.03% max.  |
| Total elements other than Mg, Al, and Mn | 0.3% max.   |
| Magnesium                                | Balance     |

The above alloy is then die cast and it has been found that by subjecting the die casting to a higher annealing temperature than customarily used for annealing or aging, and reducing the time at such temperature, a maximum amount of precipitation of the intermetallic chemical compound of aluminum-magnesium could be obtained. This resulted in increased yield strength and hardness of castings of this alloy so treated, as compared to mechanical properties obtained by conventional heat treatment times and temperatures. The exact temperature and time used in this new heat treatment is four hours at 475° Fahrenheit. Good results may be obtained between the time range of three to five hours and the temperature range of 450° to 500° Fahrenheit. However, best results are attained by the use of the exact time and temperature given above.

Through this novel heat treating or artificial aging process the grain structure of the as cast condition illustrated in the drawing of Figure 1 is converted into an approximate homogeneous equi-axed structure as shown for example in the drawing of Figure 2, which materially improves the mechanical properties of the material.

The comparative mechanical properties of the same are as follows:

|                              | As Cast Condition | Heat Treated 4 hrs. at 475° F. |
|------------------------------|-------------------|--------------------------------|
| Tensile Strength, p. s. i.   | 30,000            | 32,000                         |
| Yield Strength               | 8,000             | 21,000                         |
| Elongation, percent 2 inches | 16                | 9                              |
| Impact, foot lbs.            | 14                | 10                             |
| Hardness R <sub>100</sub>    | 35                | 65                             |

Yield strength is defined as the stress at which the stress-strain curve deviates 2% from the modulus line.

From the foregoing it will be readily seen that there has been provided a novel improved magnesium alloy and novel heat treating or aging process for producing the same.

While only one form of the invention is illustrated herein, it is to be clearly understood that the invention is not to be limited thereto, but the same is to be considered merely as illustrative of the practice thereof, since the invention is not to be limited except by the appended claims.

15. What is claimed is:

1. A die cast magnesium alloy consisting of between 1.0% and 1.5% by weight of aluminum; between 0.5% and 1.0% by weight of manganese; total elements other than magnesium, manganese and aluminum not in excess of .3% by weight, and the balance of magnesium, said alloy having a substantially homogeneous equi-axed grain structure.

2. A die cast magnesium alloy consisting of between about 1.0% and about 1.5% by weight of aluminum; total elements other than magnesium and aluminum not in excess of about 1.3% by weight, and the balance of magnesium, said alloy having a substantially homogeneous equi-axed grain structure.

3. A process for heat treating a die casting of a magnesium base alloy to improve the grain structure thereof, in which said magnesium alloy contains between 1.0% to 1.5% by weight of aluminum and the balance substantially of magnesium; comprising subjecting the casting to a temperature of approximately 475° F. for approximately four hours.

4. A process for heat treating a die casting of a magnesium base alloy to improve the grain structure thereof, in which said magnesium alloy contains between 1.0% to 1.5% by weight of aluminum and the balance substantially of magnesium; comprising subjecting the casting to heat treatment at a temperature of from about 450 to about 500° F. for approximately three to five hours.

RICHARD F. HAUSER

50. References Cited in the file of this patent

UNITED STATES PATENTS

| Number    | Name           | Date          |
|-----------|----------------|---------------|
| 1,959,913 | Gann et al.    | May 22, 1934  |
| 2,029,728 | Lowry et al.   | Feb. 4, 1936  |
| 2,029,898 | Schmidt et al. | Feb. 4, 1936  |
| 2,205,851 | Hansell        | June 15, 1940 |
| 2,267,862 | Hanawalt       | Dec. 30, 1941 |
| 2,280,103 | Swartz         | Apr. 21, 1942 |

FOREIGN PATENTS

| Number  | Country       | Date                                       |
|---------|---------------|--------------------------------------------|
| 560,104 | Great Britain | Mar. 21, 1944<br>(Provisional and amended) |

65. OTHER REFERENCES

"Die Casting," by Herb, page 51, 1936.

"Metals Handbook," page 1583, Am. Soc. for Metals, 1939.

"Die Casting for Engineers," pub. by New Jersey Zinc, pages 28-31, 1942.

"Magnesium," pages 67 and 68, Am. Soc. for Metals, 1946.